

# UNITED STATES PATENT OFFICE.

FELIX CARL THIELE, OF COFFEYVILLE, KANSAS, ASSIGNOR TO CUDAHY REFINING COMPANY, OF COFFEYVILLE, KANSAS, A CORPORATION OF MAINE.

## PROCESS FOR THE MANUFACTURE OF DRYING-OILS.

1,254,866.

Specification of Letters Patent. Patented Jan. 29, 1918.

No Drawing.

Application filed August 6, 1913. Serial No. 783,237.

*To all whom it may concern:*

Be it known that I, FELIX CARL THIELE, a citizen of the United States, residing at Coffeyville, in the county of Montgomery and 5 State of Kansas, have invented certain new and useful Improvements in Processes for the Manufacture of Drying-Oils, of which the following is a specification.

I have found that the chlorids of the eye-  
10 clo-paraffins, which are obtained when petroleum or its distillates are subjected to the action of chlorin gas, split off their chlorin as hydro-chloric acid when treated with cer-  
tain metals which have an affinity for chlo-  
15 rin, in an acid solution, and the remaining organic radicals polymerize to compounds of the methene and methine series when this occurs. The process is applicable to all chlo-  
rin products of petroleum distillates con-  
20 taining material proportions of cyclo-par-  
affins and whose specific gravity does not ex-  
ceed 0.870. The metal preferably employed for this purpose is zinc either plain or coppered, though finely divided iron mixed with  
25 aluminum may be used if desired; and while acetic acid is preferred by me for acidifying the solution, on account both of its effectiveness and economy, other acids of the same group such as butyric, proprionic, iso-buty-  
30 ric and valerianic acids may be used for the purpose. Therefore, though in the following specification I have specifically described the preferred manner of practising my in-  
vention, it is to be understood that such de-  
35 scription is for the purpose of exemplification only and that my invention is defined and distinguished to the best of my ability, from the prior art so far as known to me, in the following claim without, however, re-  
40 linquishing or abandoning any part thereof.

My process may be practised in any suitable apparatus familiar to chemists and therefore it is unnecessary to show or de-  
scribe apparatus in the present case.  
45 I will now describe a specific example of my process which is as follows: 1500 parts of a kerosene which contains a material proportion of cyclo-paraffins, of a specific gravity from 0.814 to 0.818, is treated at ordinary  
50 temperatures or slightly above the same with

moist chlorin gas until the specific gravity has increased to 1.200.

If desired bromin may be substituted for chlorin in this reaction and the same ultimate product obtained, but the results are 55 not nearly as satisfactory as the products resulting from the treatment of the hydrocarbons with chlorin and they are difficult to reduce in the subsequent treatment.

The chlorinated oil obtained in the above 60 manner is washed with cold water to remove all hydro-chloric acid and free chlorin. It is then mixed with 600 parts of acetic acid, not less than 90% strong and the mixture poured on coppered, granulated zinc or zinc 65 wool. Instead of acetic acid, as above stated, other acids of the same group may be em-  
ployed but I have found that named the most satisfactory for the purpose. An evo-  
lution of hydro-chloric acid gas begins at 70 once upon the mixture of the chlorinated oil with the acetic acid and zinc, the mixture preferably being cooled if the evolution of gas becomes violent. As above stated, for the coppered or granulated zinc we may sub- 75 stitute iron mixed with aluminum, the reac-  
tion being substantially the same in each case.

As soon as the proper chemical action has commenced the mixture of chlorinated 80 oil and acetic or other acid employed ac-  
quires an almost black color. This color becomes lighter as the action proceeds until a dark amber color indicates that it is fin-  
ished. In the meantime evolution of hydro- 85 chloric acid ceases.

The liquid after cooling is removed from the excess zinc employed and washed with hot water and finally with a dilute solution of sodium carbonate. It can be filtered 90 through Fuller's earth, sawdust or other suitable material to render the oil brilliant in appearance.

The finished products of the invention are 95 oils of a specific gravity above 0.900. They are thick, slow flowing oils which dry in the air, forming dry films, and may be used to replace linseed and other vegetable oils of a drying and a semi-drying type in all their forms in the art. The oil dries in five hours 100

when exposed to a temperature of 45° centigrade. Where it is to be used for making linoleum it is further thickened by subjecting it to steam or vacuum distillation to 5 drive off certain lighter fractions contained in it.

I claim:

A process for the manufacture of drying oils which consists in treating kerosene con-

taining a material proportion of cyclo-paraffins with a halogen, acidulating the chlorinated oil so formed, and treating the mixture of acid chlorinated oil with a metal.

FELIX CARL THIELE.

Witnesses:

ETHEL BLOUNT,  
KENT TRIPLETT.

Copies of this patent may be obtained for five cents each, by addressing the "Commissioner of Patents, Washington, D. C."